

## UNITED STATES PATENT OFFICE

2,528,867

PRODUCTION OF THERMALLY HARDENABLE  
BORON-TITANIUM STEELS

Maurice J. Day, Oak Park, Ill., assignor to Carnegie-Illinois Steel Corporation, a corporation of New Jersey

No Drawing. Application June 28, 1948,  
Serial No. 35,733

1 Claim. (Cl. 75—129)

1

This invention relates to boron-containing thermally hardenable steels having improved hardenability and the method of obtaining the same.

Boron is conventionally added to thermally hardenable steels in amounts varying from .0005 to .005% to improve or increase the hardenability thereof. It is more frequently added to the low carbon steels containing less than .30% carbon

times the amount which the nitrogen exceeds .006% or  $5 \times 0.014\%$ .

The efficiency of such additions can be readily seen from the following tabulation based on steels having otherwise similar composition, except for boron and titanium. The hardenability factor clearly shows the effectiveness of the titanium.

EXAMPLE I  
Steel A—high nitrogen

| C   | Mn  | P    | S    | Si  | Ni   | Cr  | Mo  | V   | B     | N    | Ti   |
|-----|-----|------|------|-----|------|-----|-----|-----|-------|------|------|
| .16 | .76 | .012 | .009 | .19 | 1.92 | .77 | .30 | .03 | .0024 | .011 | None |

due to its greater effectiveness therein but may be and frequently is added to steels containing up to .90% carbon. However, even in the case of the low carbon steels, the effect of the boron additions varies widely, i. e., boron additions will

15 Hardenability for boron calculated to be 1.04 where 1.00 is equivalent to no effect of boron.

EXAMPLE II

Steel B—high nitrogen

| C   | Mn  | P    | S    | Si  | Ni   | Cr  | Mo  | V   | B    | N    | Ti  |
|-----|-----|------|------|-----|------|-----|-----|-----|------|------|-----|
| .14 | .90 | .008 | .007 | .30 | 1.61 | .52 | .22 | .05 | .004 | .013 | .03 |

remarkably increase the hardenability of one steel and have little or no effect on steels of generally similar composition.

It is accordingly an object of this invention to provide a uniform increase in hardenability by boron additions to thermally hardenable steels.

It is a further object to obtain maximum efficiency from boron additions to thermally hardenable steels.

It has heretofore been noted by a number of metallurgists that boron additions to steels produced in open hearth furnaces provide the desired increase in hardenability. However, boron additions make little, if any, change in this property of steels produced in electric furnaces. I have discovered that this difference in response to boron is due to the nitrogen content and that steels containing no more than .006% nitrogen will respond effectively to boron additions. I have further discovered that steels containing over .006% nitrogen may be rendered very responsive to improvement in hardenability by boron additions by adding at least .02% titanium to the molten steel prior to or simultaneously with the boron. In electric furnace steels, the nitrogen content may use as high as .02% or higher. To obtain the maximum efficiency from the titanium and boron additions to steels containing large amounts of nitrogen, the titanium should be added in amounts at least five times the amount the nitrogen content exceeds .006%. Thus for a steel containing .02% nitrogen about .07% titanium should be added, which is five

Hardenability factor for boron calculated to be 1.71 which is a satisfactory performance for boron.

I claim:

30 The method of improving the efficiency of boron additions to thermally hardenable steels containing over .006% nitrogen comprising adding at least .02% titanium to the molten steel prior to adding the boron, the titanium addition being at least five times the amount the nitrogen content exceeds .006%.

MAURICE J. DAY.

REFERENCES CITED

40 The following references are of record in the file of this patent:

UNITED STATES PATENTS

Number Name Date  
45 2,280,283 Crafts Apr. 21, 1942

OTHER REFERENCES

50 The Iron Age, September 9, 1943, pages 50 and 51. Published by the Chilton Publishing Company, Philadelphia, Pa.

Transactions; American Society for Metals, vol. 37, 1946, pages 179 to 184. Published by the American Society for Metals, Cleveland, Ohio.

55 Journal of Research of the National Bureau of Standards, vol. 39, No. 1, July 1947, page 67.

Metal Progress, August, 1947, page 262. Published by the American Society for Metals, Cleveland, Ohio.